

## UNITED STATES PATENT OFFICE

2,016,677

## ELECTRODEPOSITION OF CHROMIUM

Oskar Krämer, Leipzig, Germany, assignor to  
Theodor Haebler, New York, N. Y.No Drawing. Application May 31, 1932,  
Serial No. 614,631

7 Claims. (Cl. 204—1)

This invention relates to the electrodeposition of chromium from chromic acid in an aqueous solution.

In previously known chromium plating baths, the practically possible deposition of chromium metal ends with a presence of catalyst in excess of from 1.7 to 2 parts in 100 parts of chromic acid in a given quantity of solution; that is, with a catalyst ratio in excess of from 1.7 to 2.

10 In the solution of the present invention, however, the catalyst ratio may be greater than 2. Apparently the optimum ratio is 2.5 and the maximum 5—at current densities of from  $\frac{1}{4}$  to 1 ampere per square inch, and with temperatures 15 from 15 degrees C. to 40 degrees C.

Also, according to the present invention, an agent is employed in the bath for combating the evil effect of large accumulations of iron ions in the bath. While said agent includes a plurality 20 of elements in chemical combination for acting as a radical to combine with iron ions in the bath to form desirable iron compounds, another agent is employed in the bath to protect such radical from becoming chemically dissociated.

25 I have so far obtained best results with a bath composed as follows (per litre of solution):

|                                                                    | Grams |
|--------------------------------------------------------------------|-------|
| CrO <sub>3</sub> (chromic acid, with 25% SO <sub>4</sub> )         | 500   |
| 30 SO <sub>4</sub> (as in H <sub>2</sub> SO <sub>4</sub> )         | 12.5  |
| KC <sub>4</sub> H <sub>5</sub> O <sub>6</sub> (potassium tartrate) | 2.5   |
| KCN (potassium of cyanide)                                         | 2.5   |

The purpose of the cyanide or equivalent content of the bath is explained as follows: The bath 35 during electrodeposition of chromium, accumulates iron ions, such ions becoming troublesome upon accumulating to the extent of about 10 grams per litre of solution in highly concentrated chromic acid solutions, such as those having 400 to 500 grams of chromic acid per litre. The cyanide radical content of the bath of the present invention, however, combines with iron ions to form a new iron cyanide compound. These cyanide ions should be stabilized, as otherwise, 45 undesirable effects may occur.

Such behaviour of the cyanide radical content of the bath, by reaction thereof with oxygen, is circumvented, according to the present invention, by the addition of an agent acting to eliminate 50 such an oxidation of the cyanide as will generate the gaseous compounds just above referred to. As aforesaid, I prefer to employ the tartaric substance of KC<sub>4</sub>H<sub>5</sub>O<sub>6</sub> for such stabilization. The action of such a substance is as follows: The acid radical thereof (C<sub>4</sub>H<sub>4</sub>O<sub>6</sub>) com-

bines with the oxygen anions to form formic acid (HCOOH). Thereby, these anions are prevented from exercising their great affinity for the individual elements of the carbon-nitrogen radical of cyanide, to break up said radical to form NO<sub>2</sub> and CO<sub>2</sub>. As a consequence, the CN is maintained to form, with iron ions in the bath, FeCN<sub>6</sub> ferric cyanide; and to form, with the iron ions and the K in the bath, while the current is off, K<sub>3</sub>Fe(CN)<sub>6</sub>, potassium ferric cyanide.

10 Regarding the iron contents which is permissible in the bath it should be noted that a certain iron content not exceeding an upper limit of about 20 grams per litre may be even advantageous in increasing the current yield and the 15 like. To a bath which is altogether free from iron I may even add some soluble iron salts, or I may use the bath in a preparatory electrolysis with iron anodes so as to electrolytically dissolve some iron therein.

20 In such a case the agent capable of precipitating the iron should not be added at once, but only after such a period of operation, that the bath contains an excess of iron above the limit mentioned above.

25 A similar beneficial influence is exerted by small quantities of other metals of the iron group, for instance nickel and cobalt, which should be used in a chemically equivalent proportion. Instead of the potassium tartrate mentioned above 30 other salts of organic acids or even the corresponding acids themselves can be used, especially so, if they are capable of forming complex chromium salts or complex chromium-iron, chromium-nickel or chromium-cobalt salts. These 35 salts permit an increased sulfuric acid content of the bath.

Various changes may be made in the details disclosed in the foregoing specification without departing from the invention or sacrificing the 40 advantages thereof.

In the claims affixed to this specification no selection of any particular modification of the invention is intended to the exclusion of other modifications thereof and the right to subsequently make claim to any modification not covered by these claims is expressly reserved.

I claim:

1. A chromic acid bath for electrodeposition of chromium having in solution during electrolysis, 50 chromic acid and more than two per cent. of sulphate radical or equivalent based on the amount of chromic acid in solution, and also approximately one-half of one per cent. of KCN and one-half per cent. of KC<sub>4</sub>H<sub>5</sub>O<sub>6</sub>.

2. The method of conducting the electrodepositing of chromium from solutions of chromic acid, which comprises establishing a bath of chromic acid, sulfuric acid, and a soluble salt of a metal of the group comprising iron, nickel and cobalt, and during the passage of electric current through said bath, maintaining the chromic acid contents and the sulfuric acid radical contents of the bath, at a ratio of 100 parts chromic acid to 2.0-5.0 parts sulfuric acid radical. 5
3. The method of conducting the electrodepositing of chromium from solutions of chromic acid, which comprises establishing a bath of chromic acid, sulfuric acid, and a soluble salt of a metal of the group comprising iron, nickel and cobalt, controlling the contents of the solution of dissolved metal of the group comprising iron, nickel and cobalt to maintain a content not above 20 grams per litre during the passage of electric current through said bath maintaining the chromic acid content and the sulfuric acid radical content at a ratio of 100 parts chromic acid to 2.0-5.0 parts sulfuric acid radical. 10
4. The method of conducting the electrodepositing of chromium from solutions of chromic acid, which comprises establishing in the bath and maintaining therein during electrolysis chromic acid, acid radical and a complex organic chromium compound of the character which results from the introduction into the bath of a substance such as potassium tartrate and maintaining in the bath during electrolysis a ratio of 100 parts chromic acid to 2.0-5.0 parts acid radical. 15
5. The method which comprises electrodepositing chromium from solutions of chromic acid in a bath containing  $\text{SO}_4$  or an equivalent, reducing said chromic acid, and, simultaneously with the carrying out of the said plating operation, providing in the bath a non-gaseous plural-element agent constituted of elements having an affinity for oxygen as in the case of potassium cyanide, said agent being capable of combining as such with the metal in the bath and protecting said agent against forming gas by combinations of one or more of its component elements with oxygen anions resulting from the electrolysis 20 maintaining in the bath during the electrolysis a second agent which as in the case of potassium tartrate has a greater affinity for the said oxygen anions than have any of the elements of the plural-element agent and, during the passage of electric current through said bath, maintaining the chromic acid content and the sulfuric acid radical content of said bath at a ratio of 100 parts chromic acid to 2.0 to 5.0 parts sulfuric acid radical. 25
6. The method which comprises conducting the electrodepositing of chromium from solutions of chromic acid in a bath containing  $\text{SO}_4$  or an equivalent, reducing said chromic acid, and, simultaneously with the carrying out of the said plating operation, providing in the bath a soluble salt of a metal of the group comprising iron, nickel, and cobalt, and also a non-gaseous plural-element agent constituted of elements having an affinity for oxygen as in the case of potassium cyanide, said agent being capable of combining as such with the metal in the bath and protecting said agent against forming gas by combinations of one or more of its component elements with oxygen anions resulting from the electrolysis 30 maintaining in the bath during the electrolysis a second agent which as in the case of potassium tartrate has a greater affinity for the said oxygen anions than have any of the elements of the plural-element agent and, during the passage of electric current through said bath, maintaining the chromic acid content and the sulfuric acid radical content of said bath at a ratio of 100 parts chromic acid to 2.0 to 5.0 parts sulfuric acid radical. 35
7. The method which comprises conducting the electrodepositing of chromium from solutions of chromic acid in a bath containing  $\text{SO}_4$  or an equivalent, reducing said chromic acid, and, simultaneously with the carrying out of the said plating operation, providing in the bath a soluble salt of a metal of the group comprising iron, nickel, and cobalt, and also a non-gaseous plural-element agent constituted of elements having an affinity for oxygen as in the case of potassium cyanide, said agent being capable of combining as such with the metal in the bath and protecting said agent against forming gas by combinations of one or more of its component elements with oxygen anions resulting from the electrolysis 40 by maintaining in the bath during the electrolysis a second agent which as in the case of potassium tartrate has a greater affinity for the said oxygen anions than have any of the elements of the plural-element agent and, during the passage of electric current through said bath, maintaining the chromic acid content and the sulfuric acid radical content of said bath at a ratio of 100 parts chromic acid to 2.0 to 5.0 parts sulfuric acid radical and also controlling the content of the solution of dissolved metal so as to maintain said content at not above 20 grams per litre. 45

OSKAR KRÄMER.

55